

1

2,886,436

## 5-AMINO-8-HYDROXYQUINOLINES AS COUPLING COMPONENTS FOR AZINE DYE IMAGES

Willy A. Schmidt, Binghamton, and Robert F. Coles, Vestal, N.Y., assignors to General Aniline & Film Corporation, New York, N.Y., a corporation of Delaware

No Drawing. Application February 21, 1957  
Serial No. 641,481

5 Claims. (Cl. 96—55)

The present invention relates to 6-amino-8-hydroxy-quinoline color formers which are particularly adapted for the production of magenta azine dyestuff images during color development of an exposed silver halide emulsion with a conventional color developer of the p-phenylenediamine class, and to a process of producing such azine dyestuff images.

It is recognized that 8-hydroxyquinoline, like any of the phenols when used as a color former for the production of dye images by color development customarily yields blue to blue-green quinonimines with the oxidation products of a p-phenylenediamine color developer. On the other hand, the 8-hydroxyquinolines are known to produce azine dyestuff images where the color developer is a triamine rather than a diamine, specifically a 4,6-diamino metanilic acid and, in this connection, reference may be made to U. S. Patents 2,486,440; 2,524,741; 2,579,420 and 2,524,725. These magenta azine dye images are of importance because of their greater brilliance and stability than the magenta quinonimine dye images obtained in the usual fashion by coupling of a pyrazolone with the oxidation products of a p-phenylenediamine.

It has been suggested that azine dye images be produced with the conventional p-phenylenediamine developers as may be seen from a reference to U.S. Patents 2,536,010 and 2,543,338. In the earlier patent, however, the color former which is used to produce the azine dyes is an aromatic phenol containing in the meta-position to the hydroxyl group, a sulfonyl amino group. After color forming development to produce the usual quinonimine dye, a ring closure is effected with elimination of the sulfonyl radical attached to the amino nitrogen atom.

In the latter patent, the color formers used are aromatic amines which contain in the meta-position to the amino group, an arylamino group or a cyano- or acylamino group. Here again, after formation of the usual quinonimine, ring closure takes place through elimination of the substituents on the amino nitrogen atom, meta to the amino group.

In each case, it is evident that, on the nitrogen atom in meta-position to the hydroxyl or amino group, there is present, a substituent group which is readily cleaved to permit ring closure to the azine.

A further method for producing azine dye images by resort to the conventional p-phenylenediamine developers is described in U.S. Patent 2,701,766. According to this patent, the color former is a 6-halogen-8-hydroxyquinonimic acid which, during color forming development, reacts with the oxidation products of the p-phenylenediamine to produce a quinonimine dye image. The quinonimine dye image then reacts with an additional molecule of the developer oxidation products with elimination of the halogen atom in 6-position to effect ring closure to an azine dye. In this procedure, it is recommended that an alkaline bath be employed to promote elimination of the halogen atom in the 6-position and ring closure to the azine.

2

We have now discovered that it is possible to produce magenta azine dye images directly and without the use of any auxiliary baths by color development with a p-phenylenediamine developer providing that there is employed, as the color former, a 6-amino-8-hydroxyquinoline in which the amino group is secondary or tertiary and contains replaceable hydrogen or an acyl or sulfonyl group. Photographic emulsions, and p-phenylenediamine developers containing such color formers, and the processing of exposed silver halide emulsions with p-phenylenediamine developers in the presence of such color formers to produce magenta azine dye images constitute the purposes and objects of our invention.

The color formers contemplated for use herein are typified by the following structure:



in which W is alkyl, such as methyl, ethyl, propyl, butyl, amyl, decyl, dodecyl, tetradecyl and the like; hydroxy-alkyl, such as hydroxymethyl, hydroxyethyl and the like; carboxyalkyl, such as carboxymethyl, carboxyethyl and the like; sulfoalkyl, such as sulfomethyl, sulfoethyl and the like; or aryl of the benzene series such as phenyl, alkyl-phenyl, i.e., tolyl ethylphenyl and the like; alkoxyphenyl, such as methoxyphenyl, ethoxyphenyl and the like; carboxyphenyl, sulfophenyl and the like, and Y is hydrogen, acyl such as acetyl, propionyl, butyryl, benzoyl and the like or sulfonyl such as methyl sulfonyl, ethyl sulfonyl, phenyl sulfonyl and the like, A is hydrogen, carboxyl or carbamino, i.e.,  $-\text{CONH}_2$  or  $\text{CONHR}$  in which R is an alkyl radical as above or a sulfonated aromatic radical containing an aliphatic radical of at least five carbon atoms, B is hydrogen, alkyl as above or an aromatic radical of the benzene series as above and C is hydrogen, hydroxy, carboxy, alkyl as above, or an aromatic radical of the benzene series as above.

Examples of color formers within the ambit of the above formula are the following:





All of the above compounds may be prepared by well known reactions. Typically, Compound 1 may be prepared as follows:

A solution of 2-phenyl-6-chloro-8-hydroxyquinoninic acid (15 gms., 0.05 mole) in 50 mls. of water containing sodium hydroxide (2 gms., 0.05 mole) was treated with ethanolamine (3.5 mls., 0.058 mole) calcium carbonate (2.5 gms., 0.05 mole) and a trace of copper sulfate and copper bronze powder. The mixture was heated at 175° in an autoclave for 10 hours. After the reaction period, the insoluble material was removed by filtration and the filtrate acidified with hydrochloric acid. The brown solid was collected and washed with water. The solid was extracted twice with 100 ml. portions of hot methanol and the residue discarded. After dilution of the extract with water and heating to coagulate the solid, the product was collected. The solid was finally dissolved in dilute bicarbonate solution and re-isolated by acidification with hydrochloric acid.

The other six substituted 8-hydroxyquinolines specifically listed may be prepared by reacting the selected amine with a 6-haloquinoline in an autoclave at 150-200° for 4 to 10 hours in the presence of a copper catalyst. Thus, n-butylamine is reacted in this way with 6-chloro-8-hydroxy-2-phenylcinchoninic acid or p-anisidine with 6-chloro-8-hydroxy-2-methylcinchoninic acid to yield Com-

pounds 6 and 8 respectively. In a similar manner, ethylamine is reacted with 6-bromo-8-hydroxyquinoline to yield Compound 9 and methylamine reacted with 6-chloro-8-hydroxyquinoninic acid to yield Compound 7.

A conversion of the secondary amine to amides or sulfonamides is effected by reaction of the amine with an appropriate carbonylchloride in the presence of an acid binding agent such as pyridine or triethylamine. The product is then isolated by the removal of the solvent at reduced pressure and acidification of the residue after dilution with water.

The 4-carboxamides, as in Compound 3 are prepared by treatment of a mixture of 6-amino-2-myristoylaminotoluene-4-sulfonic acid and 6-(methylaminobenzenesulfonamide)-8-hydroxy-2-methylcinchoninic acid in pyridine solution with one-half mole of phosphorous trichloride.

In our procedure, the azine dye image is produced from the originally formed quinonimine through elimination of the elements of acyl or sulfonyl from the amino group ortho to the intermediate azomethine coupled position in the quinoline nucleus and elimination of hydrogen from the benzene ring ortho to the primary amino group originally present in the developer molecule. Such ring closure is schematically represented by the following equation:



in which W and Y have the values given above and R' is methyl, ethyl, propyl, hydroxyethyl or the like.

It will be seen from this equation that, due to the particular structure of the color former, only one molecule of the oxidized developer is utilized in the formation of the azine rather than two molecules as in the procedure envisaged in U.S. Patent 2,701,766.

The invention is further illustrated by the following examples.

#### Example I

A color developing solution is prepared as follows:

|                              | Gms. |
|------------------------------|------|
| p-Aminodiethylaniline        | 2    |
| Sodium carbonate (anhydrous) | 50   |
| Sodium sulfite (anhydrous)   | 2    |
| Potassium borate             | .2   |
| Water to make 1 liter.       |      |

0.1 gram of Compound 1 was dissolved in 5% sodium carbonate solution (5 mls.) and the solution was made up to 50 mls. with a portion of the aforesaid color developer solution.

A strip of exposed positive film is agitated in this solution for 5 to 10 minutes. The film on which a green azomethine dye is originally produced is bleached in fer-

ricyanide and fixed in acid hypo. On treatment with the acid hypo, the green azomethine dye converts to a brilliant magenta azine dye.

*Example II*

Fifteen grams of Compound 3 were dissolved in 300 mls. of aqueous alcoholic sodium hydroxide solution and the solution added to 1 kg. of a melted gelatino-silver bromide emulsion. The emulsion was coated on film and dried.

The emulsion was exposed and color developed in the developer of Example I for 5 to 10 minutes. Upon bleaching in ferricyanide and firing in hypo, a brilliant magenta azine dye image is obtained.

Modifications of the invention will occur to persons skilled in the art. Thus, in lieu of the couplers mentioned in Examples I and II, any of the compounds listed above may be utilized for our purpose. Where the couplers are to be employed in the emulsion, they should contain a non-diffusing group, preferably an alkyl chain of at least 10 carbon atoms as per Compound 3. If, on the other hand, they are to be used in the developer, they should not possess groups which render them non-diffusing in the emulsion.

It is equally evident that, in lieu of the p-aminodietylaniline of Example I, other p-phenylenediamines may be used as, for example, 4-diethylaminoaniline, 4 - dipropylaminoaniline, 4 - (N-methyl-N-hydroxyethylamino)aniline, 4-(N-ethyl-N-hydroxyethylamino)aniline, and 4-(N,N'-dihydroxyethylamino)aniline.

We, therefore, do not intend to be limited in the patent granted except as necessitated by the appended claims.

We claim:

1. Process of producing magenta azine dye images which comprises exposing to light a light sensitive silver halide emulsion and developing the same with a p-phenylenediamine developer in the presence of a color former of the following formula:



wherein W is selected from the class consisting of alkyl, hydroxyalkyl, carboxyalkyl, sulfoalkyl, and aryl of the benzene series, Y is selected from the class consisting of

hydrogen, acyl and sulfonyl groups. A is selected from the class consisting of hydrogen, carboxyl and carbamino groups, B is selected from the class consisting of hydrogen, alkyl and aryl of the benzene series, and C is selected from the class consisting of hydrogen, hydroxy, carboxy, alkyl and aryl of the benzene series.

2. The process as defined in claim 1 wherein the color former is 2-phenyl-6-( $\beta$ -hydroxyethylamino)-8-hydroxy-cinchoninic acid.

10 3. A light sensitive silver halide emulsion containing as a color former for magenta, the compound of the following formula:



15 wherein W is selected from the class consisting of alkyl, hydroxyalkyl, carboxyalkyl, sulfoalkyl and aryl of the benzene series, Y is selected from the class consisting of hydrogen, acyl and sulfonyl groups, A is selected from the class consisting of hydrogen, carboxyl and carbamino groups, B is selected from the class consisting of hydrogen, alkyl and aryl of the benzene series, and C is selected from the class consisting of hydrogen, hydroxy, carboxy, alkyl and aryl of the benzene series.

20 4. The light sensitive silver halide emulsion as defined in claim 3 wherein the color former contains a long chain alkyl radical rendering it non-diffusing in the emulsion.

25 5. A light sensitive silver halide emulsion containing as a color former for magenta, a compound of the following constitution:



References Cited in the file of this patent

UNITED STATES PATENTS

50 2,701,766 Hensley Feb. 8, 1955

UNITED STATES PATENT OFFICE  
CERTIFICATE OF CORRECTION

Patent No. 2,886,436

May 12, 1959

Willy A. Schmidt et al.

It is hereby certified that error appears in the printed specification of the above numbered patent requiring correction and that the said Letters Patent should read as corrected below.

Column 2, line 36, for "CONHR" read -- -CONHR --; column 5, line 13, for "firing" read -- fixing --.

Signed and sealed this 31st day of May 1960.

(SEAL)

Attest:

KARL H. AXLINE  
Attesting Officer

ROBERT C. WATSON  
Commissioner of Patents